

Feb. 9, 1932.

R. B. ROBERTSON  
INTERRELATED EXTRACTING AND PULP FORMING  
PROCESS AND APPARATUS THEREFOR  
Filed April 26, 1929

1,844,600



Inventor:

Reuben B. Robertson

By Byrnes, Townsend & Brickenstein

his Attorneys.

Patented Feb. 9, 1932

1,844,600

# UNITED STATES PATENT OFFICE

REUBEN B. ROBERTSON, OF ASHEVILLE, NORTH CAROLINA, ASSIGNOR TO THE CHAMPION FIBRE COMPANY, OF CANTON, OHIO, A CORPORATION OF OHIO

## INTERRELATED EXTRACTING AND PULP-FORMING PROCESS AND APPARATUS THEREFOR

Application filed April 26, 1929. Serial No. 358,352.

The present invention is concerned with a process of extracting a tanning substance from a fibrous material containing the same, and simultaneously preparing such material 5 in the form of a pulp suitable for use in making paper or the like, and with a system of apparatus for carrying out the interrelated process. More particularly, my invention finds application to an extraction treatment 10 of a fibrous material,—such for example, as the woody parts or/and bark of oak, hemlock, and chestnut,—containing water-soluble constituents adapted for use as tanning agents, whereby the fibrous material 15 after extraction is in the condition of, and possesses the characteristics necessarily inherent in a web-forming pulp.

According to the process heretofore known and used, the raw fibrous material containing 20 water-soluble tanning agents, in its natural, relatively dry, condition, was first reduced by mechanical means to a comminuted state and the comminuted material was extracted by being brought into contact with 25 water on the principle of counter-current flow; i. e., the material was brought successively into contact with aqueous liquid containing less and less of the tanning agent in solution and finally with pure water.

In order to secure, in a reasonable length 30 of time, an adequate degree of removal of the tanning agents present in the fibrous material, it has been considered necessary to bring the material to a relatively fine state 35 of comminution. It has been the practice to maintain the extractant at any suitable temperature favorable to the production of an extract of a desired degree of purity. In those cases where the extractant was maintained 40 at a temperature at or above 212° F., the extraction was effected in pressure containers; at working temperatures below 212° F. open tanks or tubs were employed.

This fine sub-division of the fibrous material in its natural, relatively dry, state resulted in the production of a product containing a large proportion of powdered material and of fibrous particles in which the ultimate fibers and fiber bundles were greatly shortened, with the result that, after extract-

tion, the by-product fibrous material no longer had value as a raw material for paper pulp.

An object of the present invention is the provision of an inter-related tannin-extracting and paper pulp-forming process by the carrying out of which a tanning substance may be extracted from a fibrous material containing the same, and the said fibrous material may simultaneously be prepared in the form of a pulp suitable for use in making paper or the like.

My new process comprises the steps of partially or coarsely comminuting the raw fibrous material, subjecting the coarsely comminuted material to treatment with an aqueous extractant, refining the treated material and subjecting the same to contact with an aqueous liquid, and thickening and washing the re-treated material. A feature of the process consists in washing the thickened material with an amount of water calculated to replace the water lost from the system in the extract and in the washed material, and the use of this wash water in the system for making up said losses.

The fibrous material undergoing the first extraction treatment is in a state of comminution sufficiently coarse-fibered to avoid material cutting or shortening of the fibers or fiber bundles. The refining treatment is effected upon the material after the fibers and fiber bundles have become softened, hence the refining treatment tends to separate the fibers of the bundles rather than to cut or rupture them. When refined and treated in this manner, the resulting product is in a most favorable condition for use as a paper-making pulp. In fact, a feature of the invention consists in effecting the thickening operation by forming the refined material into a sheet, on an appropriate thickening and sheet-forming device such as, for example, a continuous suction thickener, on the cylinder mould of a paper machine or the like, of any convenient type, and washing the material with the fresh water while said material is in the sheet form.

The cyclic nature of my process becomes apparent by tracing the water used in washing the thickened material, disregarding the

water remaining in the material after the washing operation; the wash water is used partially in the refining operation, and partially as aqueous extractant in the extraction operations. There thus is accomplished the substantially complete saving of water-soluble tanning substances, with a minimum dilution of the extract. The process has the further advantage that it provides for complete elimination of the necessity for discharging, to the sewer, waste water containing appreciable quantities of the tanning agents, and therefore aids in the effort to maintain the public water in a relatively high degree of purity.

The invention will be explained more fully by reference to the accompanying drawing, which is a diagrammatic representation of an operable embodiment of the process and of an operable system of apparatus.

In the drawing are represented, in a closed system, in addition to the necessary piping, valves, and the like, a plurality of leach tanks 1 to 12, inclusive, a refiner 13, a diffusing means 14, a web-forming device 15, a pump 16, a dilute liquor storage 17, a pump 18, and a heating means 19. 20 is a coarse comminutor. The leach tanks, 1 to 12, inclusive, may be either of the open, or pressure type, depending primarily upon whether the first extraction operation is to be effected at below or above the boiling point. The said tanks are so arranged and so coupled by means of suitable piping, valves, and the like, as indicated, that an aqueous extractant, e. g., water, or wash water, can be introduced into any one tank, as into leach tank 10 in the accompanying diagram, thereafter flow continuously, as indicated, through tanks 9, 8, etc., and, after passing through a plurality of the leach tanks, e. g., through tanks 10 to 3, inclusive, as indicated, be discharged, as at tank 3, from the system and run to evaporators (not shown). The refiner 13, which may be any suitable known means for opening up softened fiber bundles of pulpable fibrous material, in the presence of an aqueous liquid, such as, for instance, a rod mill or a refiner of the "Jordan" or "Claflin" types, is interposed between the leach tanks 1 to 12, inclusive, and the diffuser 14 and is connected thereto by any suitable piping. The diffusing means 14 may take the form of a tank, or series of tanks (either open or closed, as desired), which tank or tanks conveniently may be, and preferably are, provided with some suitable means of agitation. The purpose of the tank or tanks 14 is to provide, in a continuously operated system, a period of contact between aqueous extractant and refined fibrous material sufficient to insure adequate extraction of tanning agents not already extracted in the leach tanks 1 to 12, inclusive. The web-forming device 15 may be any suitable known device for simultaneously thickening and forming

a sheet or web, such, for instance, as the cylinder mould of a paper-making machine, or the like. The heating means 19 likewise may be any known and suitable device for transmitting heat to a liquid.

In operation, the leach tanks will contain coarsely comminuted fibrous material having progressively decreasing contents of water-soluble tanning substances; in one or more of the tanks, as 11 and 12 in the diagram, there will be fibrous material which is practically exhausted as to readily available tanning content, which material is being removed to the refiner 13 while one or more of the tanks, as 1 and 2 in the diagram, will be being charged with fresh coarsely comminuted fibrous material; in the intermediate leach tanks will be material undergoing the first leaching treatment with the dilute aqueous liquor from storage 17, said liquor first contacting with the nearly exhausted material in tank 10 and thereafter being brought successively into contact with material containing progressively larger proportions of the tanning substances. The resulting relatively concentrated aqueous solution of tanning substances,—i. e., the extract, or "strong liquor",—is withdrawn from the system after passing through tank 3 which contains fresh material for evaporation. When tanks 11 and 12 have been emptied of their charge of relatively exhausted fibrous material and tanks 1 and 2 have been charged with fresh material, the tanks 10 and 9 are cut out of the system, for discharge to the refiner 13, the aqueous extractant from storage 17 then being introduced into the system of leach tanks first at tank 8, and passing through tanks 8 to 1, inclusive, before withdrawal to evaporation.

The relatively exhausted fibrous material discharged from the system of leach tanks is passed in a stream through the refiner 13 in association with dilute liquor from storage 17, the fiber bundles of the fibrous material being opened up so as to bring the same into the condition of a pulp suitable for use in making paper. The resulting stream of refined material in suspension in the liquor is then caused to pass into and through the diffuser 14 where the flow of pulp suspension is retarded to provide a period of contact between the dilute liquor and the refined material adequate to effect thorough extraction of the tanning substances made available in the material by the refining operation.

The pulp suspension of refined and finally exhausted fibrous material flows from diffuser 14 to the web-forming device 15 where it is thickened in the known manner and simultaneously formed into a sheet or web, and is washed thereon, in the form of a sheet, with a predetermined amount of fresh water. In the operation of thickening and washing, the weak liquor separated from the pulp is com-

bined with the wash water from the washed pulp. The amount of fresh water added is that required to replace the net amount of water leaving the system in association with (1) the thickened and sheeted pulp and (2) the extracted tanning substances in the strong liquor withdrawn from the system of leach tanks.

The weak wash liquor and wash water from the web-forming device 15, containing in dilute solution tanning substances washed out of refined material, is withdrawn by means of pump 16 to dilute liquor storage 17, from which it is distributed, by pump 18, to several points in the cycle. One portion of dilute liquor is returned directly to the pulp suspension from diffuser 14—for diluting the same to a consistency suitable for application to the thickener. A second portion of dilute liquor is passed through the heating means 19 and delivered in part to the refiner 13 and in part to the system of leach tanks 1 to 12, inclusive. In case the said leach tanks are of the pressure type, a portion of the dilute liquor may by-pass the heater to the refiner; in such a case hot liquor from the heater is delivered to the refiner in a quantity sufficient, when mixed with the unheated liquor, to give the entire mass the desired temperature.

It will be seen that the process is substantially continuous and in a closed cycle of operations; that all of the tanning content of the fibrous material is conserved in the form of a relatively concentrated extract; that the fibrous by-product material is recovered in the form of a paper-making pulp; and that neither tanning substance nor fiber is discharged to waste. The process is simple; it requires a minimum amount of handling of material, of power and of labor. The system of apparatus is of an economical character.

I claim:

1. A process for recovering water-soluble tanning substances from raw fibrous material containing the same and for simultaneously preparing said material in the form of a paper web, which includes the following steps: (a) subjecting the raw fibrous material in coarsely comminuted form to preliminary extraction with aqueous liquid obtained from step (e) and separating the preliminarily extracted material from the resulting extract of water-soluble tanning substances; (b) refining the separated material from step (a) in the presence of aqueous liquid obtained from step (e) and subjecting it to prolonged diffusion treatment in said liquid; (c) thickening the diffused material and simultaneously forming the same into a paper web while retaining the aqueous liquid separated therefrom; (d) washing the web with water; and (e) combining the wash water

from step (d) with the separated aqueous liquid from step (c).

2. A process for recovering water-soluble tanning substances from raw fibrous material containing the same and for simultaneously preparing said material in the form of a paper web, which includes the following steps: (a) subjecting the raw fibrous material in coarsely comminuted form to preliminary extraction with heated aqueous liquid obtained from step (e) and separating the preliminarily extracted material from the resulting extract of water-soluble tanning substances; (b) refining the separated material from step (a) in the presence of heated aqueous liquid obtained from step (e) and subjecting it to prolonged diffusion treatment in said liquid; (c) diluting the diffusion mass with aqueous liquid obtained from step (e), thickening the diffused material and simultaneously forming the same into a paper web while retaining the aqueous liquid separated therefrom; (d) washing the web with water; and (e) combining the wash water from step (d) with the separated aqueous liquid from step (c).

3. A process for recovering water-soluble tanning substances from raw fibrous material containing the same and for simultaneously preparing said material in the form of a paper web, which includes the following steps: (a) subjecting the raw fibrous material in coarsely comminuted form to preliminary extraction with heated aqueous liquid obtained from step (e) and separating the preliminarily extracted material from the resulting extract of water-soluble tanning substances; (b) refining the separated material from step (a) in the presence of heated aqueous liquid obtained from step (e) and subjecting it to prolonged diffusion treatment in said liquid; (c) diluting the diffusion mass with aqueous liquid obtained from step (e), thickening the diffused material and simultaneously forming the same into a paper web while retaining the aqueous liquid separated therefrom; (d) washing the web with an amount of fresh water equal to the total water leaving the system in the water-wet web and in the extract obtained in step (a); and (e) combining the wash water from step (d) with the separated aqueous liquid from step (c).

4. The process as defined in claim 1, characterized in that the extraction operation in step (a) is effected under superatmospheric pressure and at a temperature at least equal to the boiling point of water.

5. A system of apparatus for simultaneously and continuously extracting tanning substances from fibrous material containing the same and preparing the material in the form of a paper web by the process substantially as described, which comprises means for partially extracting fibrous material and means for delivering coarsely comminuted material

thereto, a refiner receiving extracted material from said first named means, means for forming into a web the refined material delivered thereto from the refiner and for washing the web, and means for delivering liquid from said web-forming and washing means to said extraction means and to said refining means.

6. A system of apparatus for simultaneously and continuously extracting tanning substances from fibrous material containing the same and preparing the material in the form of a paper web by the process substantially as described, which comprises means for partially extracting fibrous material and means 15 for delivering coarsely comminuted fibrous material thereto, a refiner receiving extracted material from said first named means, means for forming into a web the refined material and for washing the web, a diffuser receiving 20 material from said refiner and delivering material to said web-forming and washing means, and means for delivering liquid from said web-forming and washing means to said extraction means and to said refining means.

25 In testimony whereof, I affix my signature.

REUBEN B. ROBERTSON.

30

35

40

45

50

55

60

65